

## UNITED STATES PATENT OFFICE.

WILLIAM J. MERTEN, OF PITTSBURGH, PENNSYLVANIA, ASSIGNOR TO WESTINGHOUSE ELECTRIC & MANUFACTURING COMPANY, A CORPORATION OF PENNSYLVANIA.

## QUENCHING BATH.

No Drawing.

Application filed May 4, 1925. Serial No. 28,014.

To all whom it may concern:

Be it known that I, WILLIAM J. MERTEN, a citizen of the United States, and a resident of Pittsburgh, in the county of Allegheny and State of Pennsylvania, have invented a new and useful Improvement in Quenching Baths, of which the following is a specification.

10 My invention relates to a composition of matter and more specifically to a quenching bath for use in the heat treatment of steel.

It is among the objects of my invention to provide a quenching bath that will quickly and uniformly cool the heated specimen in such manner that soft spots or hair-like cracks are not formed in the steel.

15 It is the practice in making objects of steel, such as tools, to forge the material into the desired shape and then to harden the steel by heating to the desired temperature and quenching. A fused salt bath is one of the commonly used means for heating the steel, as the temperature of the same is readily controlled and because the steel is 20 protected from oxidation and decarbonization during heating. Baths ordinarily used for quenching are either water, lime, oil or a solution of sodium chloride in water and sulphuric acid. When any of the above 25 baths are used for quenching after having been heated in fused salt mixtures, the steel develops hair-like cracks and soft spots in the surface thereof.

Heretofore, it has been believed that such 30 defects were caused either by the lack of uniformity in the composition of the steel or by reason of uneven heating and decarburization of the steel. I have discovered that the defects are results of the uneven 35 cooling when the steel is quenched.

When steel is quenched in the baths hitherto used, the steel is protected by a film of oxide or gas or other heat non-conducting material, so that certain small areas in the 40 specimen are cooled less rapidly than the rest of the specimen. For example, a dense troostitic structure is formed in one small area and a less dense martensitic structure occurs in the immediate adjoining area. 45 Therefore, enormous internal stresses are developed in the steel. The excessive stress in the less dense martensitic area is conducive to a change of structure to the more stable and more dense troostitic condition

and, as a result, hair-like cracks and checks 55 occur in the surface of the steel. A finish grinding operation, which produces local heating, is particularly likely to develop such defects. The development of soft spots in the steel is also caused by the lack of uniformity in conducting the heat away from the steel in the quenching bath. The lack of uniformity in conducting heat from the steel is the result of films of gas and surface 60 oxides of low heat conductivity and also of 65 surface films of salts or highly concentrated solutions thereof having low heat conductivity.

My invention provides a quenching bath 70 which instantly dissolves adhering salt on the steel and prevents the formation of vapor, gas or oxide films of low heat conductivity. When the steel is immersed in the bath it is quickly and uniformly cooled and the resulting surface is free from soft 75 spots and hair-like cracks.

I provide a bath containing a combination 80 of constituents which react with the vapors and non-conducting films on the surface of the steel to dissolve, eliminate and prevent the formation of heat insulators or non-conductors as fast as they are formed. I prefer a bath of the approximate composition: water 48%, sodium chloride 24%, lime 85 16%, sodium cyanide 12%.

In use, the bath is agitated to keep the lime in suspension. When steel is quenched 90 in this bath, not even a slight oxidation of the surface occurs on the steel, and the steel retains its original lustre.

Although I have described a specific bath 95 embodying my invention, I do not wish to be limited thereto, as the proportions of the several constituents may be modified. For example, I vary the proportion of lime and an alkali cyanide from 5 to 20%, of an alkali chloride from 15 to 24% and of water from 40 to 60%. I may also substitute potassium salts for the sodium salts and magnesium or other alkaline earth metal oxides 100 for the lime. Other modifications of my invention will suggest themselves to those skilled in the art without departing from the spirit of my invention, the scope of which is defined in the annexed claims.

I claim as my invention:

1. A quenching bath which comprises an aqueous solution of an alkali metal chloride,

2. an alkali metal cyanide and an oxide of an alkaline earth metal.
5. 2. A quenching bath which comprises an aqueous solution of a mixture of alkali metal chlorides, a mixture of alkali metal cyanides and oxides of alkaline earth metals. 15
5. 3. A quenching bath which comprises an aqueous solution of a metal chloride, a metal cyanide and a metal oxide.
- 10 5. 4. A quenching bath which comprises an aqueous solution of sodium chloride, sodium cyanide and lime. 20
5. 5. A quenching bath which comprises about 24% sodium chloride, 12% sodium cyanide, 16% lime and the remainder water.
5. 6. A quenching bath which comprises 15 to 24% of an alkali chloride, 5 to 20% of an alkali cyanide, 5 to 20% of an alkaline earth metal oxide and the remainder water.
- In testimony whereof, I have hereunto 20  
subscribed my name this 29th day of April,  
1925.

WILLIAM J. MERTEN.